

A. S. DWIGHT.  
PROCESS OF TREATING ORES.  
APPLICATION FILED JUNE 17, 1911. RENEWED JUNE 2, 1917.

1,254,316.

Patented Jan. 22, 1918.

2 SHEETS—SHEET 1.



Fig. 3



Inventor

A. S. Dwight

By H. T. Bias Attorney

Witnesses

F. L. Dodd.

S. Jay Teller

A. S. DWIGHT.

## PROCESS OF TREATING ORES.

APPLICATION FILED JUNE 17, 1911. RENEWED JUNE 2, 1917

1,254,316.

Patented Jan. 22, 1918.

2 SHEETS—SHEET 2.



Fig. 5



Fig.



Fig. 7

Witnesses

F. L. DeWitt

S. Jay Teller

**Inventor**

A. S. Dwight

By J. H. Bliss Attorney

# UNITED STATES PATENT OFFICE.

ARTHUR S. DWIGHT, OF NEW YORK, N. Y.

## PROCESS OF TREATING ORES.

1,254,316.

Specification of Letters Patent. Patented Jan. 22, 1918.

Application filed June 17, 1911, Serial No. 633,760. Renewed June 2, 1917. Serial No. 172,522.

*To all whom it may concern:*

Be it known that I, ARTHUR S. DWIGHT, a citizen of the United States, residing at New York, in the county of New York and

5 State of New York, have invented a certain new and useful Improved Process of Treating Ores, of which the following is a specification, reference being had therein to the accompanying drawing.

10 This invention relates to processes for treating metal-bearing materials which are normally in an initially fine or pulverulent condition and which do not contain native combustible elements (such as sulfur, or its equivalent) in sufficient quantities; it relating particularly to a process for the treatment of metal-bearing materials which are characterized principally by the presence of the metal oxids.

15 The oxid bodies referred to are well typified by the ores containing iron oxids, such as hematite, magnetite, limonite, etc.

20 The term "ore," as herein used, refers to mineral-bearing masses, (both those in their native conditions and those that are artificially formed) which include not only the metal oxid of one form or another, but include also other materials that are ordinarily found in these ores, such a silica, earthy bodies, or the like, and also traces, or larger quantities, of other metalliferous materials.

25 By the "iron oxid ores" (typically above mentioned), such as hematite  $Fe_2O_3$ , magnetite  $Fe_3O_4$ , or limonite  $FeO_3H_6$ , etc., reference is made to those iron ores which are, 30 respectively characterized more particularly by the presence of these oxids, even though accompanied in any given case by other ore components; and, as is well known, these 35 oxid ores are found in large quantities in a fine or pulverulent condition.

40 The reduction of any finely divided ores in a blast furnace, or similar apparatus, without preliminary treatment, involves 45 considerable difficulty and loss, because of the tendency of the fine ore particles to settle into and choke the gas passages in the mass in the furnace and because of the tendency for large quantities to be carried off by the blast and deposited as "flue dust" or scattered to points outside of the furnace.

50 These pulverulent ores may, for present

purposes, be classified as those which are of the sulfid class, and those which are of the 55 oxid class.

As concerns ores characterized by the presence of a material amount of sulfur or equivalent, combustible, I have heretofore (either solely or jointly with others) devised a process for, and have succeeded in, transforming them into agglomerated or sintered 60 blocks or cakes which can be readily introduced into the blast furnace, and which there operate in an advantageous and economical manner.

65 In that process the agglomerating or sintering of the fine ores is effected by means of heat derived from combustion of substances in chemical combination and contained therein; this combustion occurring within 70 the ore mass. The ore is distributed in a layer of stratum which is relatively thin or shallow, so that there is no material amount of weight or pressure exerted at any region and so that the air can be readily passed 75 through the layer with great uniformity on all vertical lines. The sulfur component of the fine particles is ignited at the exposed surface and its combustion is supported by the air currents which are passed through 80 the stratum from the plane of ignition toward a plane of escape. And at the region of the latter plane and throughout the mass the particles are held against agitation, or movement, in relation to each other; that is, 85 agitation such as might be caused by the air currents or otherwise.

85 The oxidizing of the sulfur (and an accompanying oxidizing of the metals) is carried on to the desired degree, some of the 90 sulfur being generally allowed to remain, and more or less of metallic oxids (as oxids of copper and iron) are produced. And, at the same time, the agglomerating is effected, 95 this latter including the reaction of the silica upon such base materials as are initially present or are formed. The gases that are generated at the time of the reactions and at the time that particles are permitted to ehere, act to form large cells or pores in 100 the nascent and softened mass, and these are uniformly distributed through the stratum from the top to the bottom; and after the instant of the forming and the

cooling of the silicated and agglomerated materials these cells or pores remain, and constitute important matters, during the stage of treatment in the blast furnace. The presence of the silicates of the basic materials, metallic or other, is not detrimental in the blast furnace, as concerns ores of the sulfid, or equivalent, classes.

In Patents Nos. 882,517 and 882,518, issued to R. L. Lloyd and myself, jointly, there are disclosed processes involving these steps.

But when I undertook to agglomerate or sinter finely divided or pulverulent ores of these other classes, to wit, those of the oxid class, or their equivalents, different conditions were met and peculiar difficulties were experienced by me. I found that the agglomerating of the fine particles of the oxid ores must depend upon activities other than those which I found to be efficient in operating on the materials of the sulfid class, and that the cementing or binding of these particles must be secured by different causes. I found, particularly, that the silicating, or the like, of the basic materials should not be depended on, and, in fact, should be avoided as far as possible.

I further discovered that in order to prevent the temperature from being raised to the point of silicification, the oxid ore should be arranged in a relatively thin layer, so that the heat, after performing the necessary work, would readily escape by conduction through short paths, and by radiation.

In place of the sulfur I employ carbonaceous material in pulverulent form, which is intimately and uniformly commingled with the ore oxid. This is ignited at the exposed surface and the combustion is carried through the mass by currents of combustion gas, such as the oxygen of the atmosphere. The carbon oxids peculiarly interact with the metal oxid and by properly controlling and regulating the different materials I am able to effect a binding of the particles together, not so much by an action like that of silicating a base material as by causing the union of one form of metal oxid with another, the oxids passing from one form to another in the presence and under the influence of the carbon oxids.

Of the accompanying drawings which form a part of this specification,

Figure 1 is a side elevation partly in cross section of one form of apparatus adapted for use in carrying out my improved process.

Fig. 2 is a plan view partly in cross section of the apparatus shown in Fig. 1.

Fig. 3 is an enlarged fragmentary cross sectional view taken along the lines 3—3 of Figs. 1 and 2.

Fig. 4 is a cross sectional view taken along the line 4—4 of Fig. 2.

Fig. 5 is a view of the preliminary mixing mechanism separate from the other parts of the apparatus.

Fig. 6 is a view showing the sintering mechanism separate from the mixing mechanism and from the furnace.

Fig. 7 shows a separate furnace into which may be fed material preliminarily treated by the mechanism shown in Fig. 4.

It will be understood that the forms of apparatus shown in the drawings have been selected merely as typical of the various forms of apparatus which may be used for this purpose, and that my invention is not limited to any particular form of apparatus. I do not herein claim as a part of my present invention either of the forms of apparatus which I have shown for the sake of illustration as these are shown and claimed in co-pending applications among which are certain applications filed by me and serially numbered 440,404, 544,507 and 558,621.

In an apparatus for carrying out my improved process a suitable mechanism is provided for effecting the mixing of the ore to be treated with a combustible substance, and when desirable or necessary with a suitable fluxing material.

In the drawings, I have indicated by A one form of mechanism which may be used for this purpose. 1 is a receptacle in which the ore to be treated is deposited. The receptacle 1 is preferably hopper-like in shape and is provided with a centrally located bottom opening. 2 and 3 are other hopper-like receptacles located adjacent the receptacle 1 and also provided with bottom openings. Mounted beneath the bottom openings of the hoppers is an endless belt 4 which is suitably mounted and connected for continuous movement in the direction of the arrow in Fig. 2. By referring to the drawings, it will be observed that the bottom openings of the hoppers are out of alignment with each other longitudinally of the belt, and that material from each hopper can be deposited on the belt without interference with material from either of the other hoppers. In operation, let it be assumed that the material to be treated, as for instance iron ore, has been deposited in the receptacle 1, that a combustible substance, preferably powdered coal, charcoal or coke when iron ore is to be treated, has been deposited in the receptacle 2, and that a fluxing material, such as crushed limestone, has been deposited, if needed, in the receptacle 3. As the belt 4 moves beneath the hoppers it draws out from each of them a continuous stream of material. The thicknesses of these streams can be regulated by adjusting the positions of the doors or slides 5, 6 and 7 which are located adjacent the belts at the front sides of the respective receptacles.

8 is a box-like trough mounted in position to receive at one end materials discharged from the moving belt 4. Inside of the trough is a continually rotating stirrer 9 having spirally arranged blades which serve not only to mix the materials in the trough but also to gradually work them toward the other end which is provided with an opening discharging into a chute 10. This chute 10 communicates at its other end with the hopper 11 to which the thoroughly mixed materials are conveyed.

B represents as a whole one form of mechanism which may be used for effecting the sintering and agglomerating step of the process. Of this mechanism 12 is an air suction box from which air is exhausted by means of a fan 13. Upon the upper edges of the box are carefully planed wearing strips 14 upon which slide cast iron pallets 15, the lower edges of which are likewise carefully planed so as to make an air tight joint with the strips when the pallets are pushed along the top surface of the box. 20 The pallets carry the grates 16 and are built with transverse members 17 which together with the sides of the pallets form four-sided boxes beneath the grates. Above the grates these transverse members are omitted so 25 that when a number of pallets are adjacent each other an uninterrupted grate surface is provided. These lower transverse members also serve as partitions to cut off the air at certain points in a manner which will be 30 described.

Each of the pallets may be considered as an independent or individual car provided with four wheels 18-18 attached by suitable bearing pins so arranged that the axes of 40 the wheels are in the same plane with the lower edges of the pallets, each pallet being thus permitted to move around the curved track hereinafter described without interference with the other pallets. As the pallets are pushed across the suction box they are guided by the flanges of the wheels 18-18 which are in engagement with the longitudinal track rails 19-19, the weight of the pallets being sustained on the wearing strips 14.

At each end of the suction box there is arranged a dead plate 20, the upper surface of which is flat and in alinement with the upper surfaces of the strips 14. The pallets 55 move with an air tight joint over the surface of one dead plate 20 just before they pass to a position over the suction box and pass with an air tight joint over the surface of the other dead plate 20 after they pass 60 the suction box. Each of these dead plates has a length slightly greater than the length of a pallet so that there will be no leakage of air during the time that a pallet is but partly over the suction box.

65 The pallets are elevated one by one and

consecutively placed in position on the rails 19-19 by means of a pair of sprocket wheels 21 which are so designed that their teeth engage the treads of the wheels 18-18 in conjunction with the guide rails 22.

At the end of the suction box which is farthest removed from the sprocket wheels 21 the track rails 19-19 are curved suddenly downward. Outside of and concentric with the curved ends of the rails 19-19 are rails 23 which are continued at a downward and backward incline at their lower ends and which join with the guide rails 22. It will be observed that as each pallet reaches the curved parts of the rails 19-19 it will move downward out of alinement with the other pallets and into position on the rails 23 for engagement by the sprocket wheels 21.

The hopper 11 which has been before referred to is mounted above the pallets 15 on the track wheels 18-18 and serves to deposit on the pallet grates a uniform layer of the materials which have been discharged from the mixing mechanism A.

As the pallets are pushed slowly forward 90 by the sprocket wheels 21 the layer of material on them is carried away from the hopper 11 and beneath an igniting device such as is indicated at 24. This igniting device serves to fire the combustible substance, such as powdered coal which has been mixed with the ore, in the manner before described. The igniting device 24 may be simply a perforated pipe adapted for supplying gas to support flames which continually play upon the top surface of the ore layer.

As the layer is farther advanced the combustion, which has been started by the ignitor 24, is caused to progress slowly downward through the mass by the action of a combustion supporting gas such as air, which is drawn downward into the suction box B through the interstices between the particles of material of which the mass is composed. The heat of combustion is sufficient to induce chemical activities or reactions which will cause constituent elements of the ore to become relatively softened at the time of nascent, and, as will be referred 110 to more fully below, with the result that they unite and harden upon cooling to form a rigid integral cake. On account of the continuous passage of the air and the formation of large quantities of the carbon oxides 120 through the cake during the process of sintering, the cake is highly and uniformly porous, and on this account well adapted for the smelting action which will be hereinafter described. It will be understood 125 that the rate of movement of the pallets along the upper track rails 19-19 is relatively slow and is so regulated, that when the combustion and sintering at any one point has progressed downward entirely 130

115  
105  
100  
110  
115  
120  
125  
130

through the layer, that point will have moved beyond the suction box and substantially to the discharge end of the machine.

In the construction shown in Figs. 1 and 5, the sintering is moved continuously forward onto a shelf 25 which is adjacent and in alignment with an aperture 26 in the wall of a smelting furnace which is indicated as a whole by C. The pallets 15 after freeing 10 themselves from the sinter cake return by gravity in the manner before described to be picked up and returned by the wheels 21.

The furnace here selected for illustration is of a reverberatory form. It is provided 15 with a hearth indicated at 27 and with a receptacle 28 adapted for the retention of molten metal or matte as indicated at 29 and a top layer of slag as indicated at 30. Tap holes 31 and 32 are provided for the 20 metal and the slag respectively. Nozzles 33 are provided to direct flames directly onto the incoming sinter cake at points immediately above the hearth 27. The fuel supplied to the nozzles 33 may be either gas or 25 oil and is conducted through the pipes 34 and 35. 36 is a flue for waste gases from the furnace, and in this flue are located pipe coils 37 and 38 which connect with the pipes 34 and 35 and serve to preliminarily 30 heat the oil or gas which is supplied to the nozzles 33.

I have described the step of adding fluxing material to the ore, when such materials are needed, as taking place in the preliminary mixing mechanism and I consider the 35 introduction of fluxing materials at that point preferable, as they are in that way brought into more intimate contact with the ore particles. However, if desired, the hopper 39 may be used for the supplying of 40 fluxing materials to the ore at points immediately adjacent the region of smelting. Obviously, if desired, fluxes can be supplied through both of the hoppers 3 and 39.

45 As the forward part of the advancing sinter cake passes within the heating zone of the flames from the nozzles 33 it is smelted into a metal or matte, while the earthen ingredients separate themselves into the 50 form of slag. The molten metal or matte being the heavier is collected in the bottom part of the receptacle 28 as indicated and the slag collects in the upper part of the receptacle 28 on top of the metal. Because 55 of the great and uniform porosity of the sinter cake it is readily attacked by the flames and is very quickly and sufficiently smelted.

60 While it is desirable that the incoming sinter cake remain unbroken until smelted it is not essential, as it is obvious that any part of the sinter cake which may accidentally break off will remain on the hearth 27 within the zone of the flames until smelted.

65 It will be observed that when the furnace

is located immediately adjacent the sintering machine as shown in Figs. 1 and 2, the sinter cake is passed to the furnace while still retaining the heat of sintering, and that as a result of this the smelting takes place 70 more rapidly than with the use of a smaller quantity of fuel than would be the case if the sinter cakes were allowed to cool before being smelted.

It is also to be borne in mind that the 75 sintering itself is a step in the process of smelting and that as a result of the sintering, the smelting is much more readily accomplished.

In the smelting of iron ores the presence 80 of carbon is necessary. The required carbon can, if desired, be supplied, instead of flux, through the hopper 39. Preferably, however, an excess of carbon beyond that necessary for sintering is added to the ore in the 85 preliminary mixing mechanism. By properly regulating the quantity of carbon supplied and by properly adjusting the draft and the rate of movement of the sintering machine, a portion of the carbon may be re- 90 tained in the sinter cake and carried by it into the furnace and intimately mixed with the ore and flux particles.

In Fig. 5, I have shown the preliminary 95 mixing mechanism A separate from the sintering mechanism. The construction is similar to that hereinbefore described, with the exception that, the material is delivered to a suitable point of storage instead of being delivered directly to the sintering machine. 100

In Fig. 6, I have shown a sintering machine separate from the mixing mechanism and from the furnace. The construction is similar to that hereinbefore described. The material from the mixing mechanism, which 105 may be at a remote point, is conveyed to the sintering machine in any desired manner and placed in the hopper 11. The forward portion of the sinter cake instead of being passed directly into the furnace is allowed 110 to break off from time to time and to collect in a pile from which it may be removed from time to time to a region of storage or directly to a smelting furnace.

In Fig. 7, I have shown a smelting furnace 115 separate from the mixing mechanism and the sintering machine. This furnace may be located, if desired, at a remote point and the sinter cakes or blocks may be supplied to it in any desired manner. The construction of the furnace is similar to that 120 which has been hereinbefore described.

It is believed that the general nature and scope of my improved process will be apparent from the foregoing description of the 125 construction and operation of the apparatus selected for purposes of illustration. However, it may be well to point out in detail the actions incident to the various steps of the process, references being had more particu- 130

larly to the use of an oxid iron ore and a carbonaceous material such as powdered coal or coke. For illustration, I will assume that the metal body to be treated is the above 5 mentioned magnetite iron ore.

The iron oxid after having been mixed with a proper quantity of powdered coal or coke and with a flux if desired, is deposited upon the moving grate of the sintering machine and the coal or coke is ignited at the top surface in the manner which has been described. Air is drawn downward through the interstices of the mixture and causes the combustion of the coal or coke to 10 progress downward and inward through the mass. The action which takes place is in some respects similar to the action which takes place in a blast furnace. The carbon in burning generates, of course, the ordinary 15 carbon oxids. The plane of combustion proceeds from the surface toward and through the interior. The atmospheric oxygen is supplied more slowly the farther the air travels inward and there tends to be a correspondingly large amount of carbon monoxid 20 generated, but this, in turn, as more oxygen is taken up by it, passes into the dioxide form; and the mass of metalliferous particles are enveloped in these carbon oxids. 25 The temperature which is generated raises that of the iron oxids to the points where reactions can occur. The magnetite, in the presence of the carbon oxids, manifests the tendency, largely from contact reaction, to 30 adhere to neighboring particles, either those of its own constitution or those of other compositions. It is an instance of the phenomenon analogous to cementation of certain forms of iron. There is, also, a tendency for 35 it, under certain conditions, to pass into other lower oxid forms, and the lower and the higher oxids, in the presence of the carbon oxids, unite again to form a ferrite. The temperature at which this occurs (from 40 45 600° to 800° C.) is much lower than that at which silicification occurs.

If in the reactions between the metal oxids and the carbon oxids any metallic iron is temporarily released, the particles of such 50 metal tend to unite and assist in establishing the coherency of the mass.

If, instead of the iron oxid ore being largely magnetite, it is of the lower oxid form, namely hematite: as soon as it is heated and enveloped in the bodies of carbon oxids more or less of it takes on more oxygen and becomes relatively acid in character, and this part in turn unites with the lower oxid and produces a ferrite which, at the 55 time of nascence, and as above described, produces a cohering analogous to cementation and at a temperature much lower than that at which the silicification of the iron occurs.

60 65 I am aware of the fact that it has been

heretofore proposed to mix carbonaceous material with iron ores and then place the mixture in a large pct or converter and with a powerful blast attempt to force air through it for the purpose of agglomerating 70 it. But, so far as I have been able to learn, no success was attained and all such attempts have been abandoned.

It was discovered that in the case of most of the iron ore bodies the fineness or pulverulency was even greater than that incident to the sulfid ores. To cause the air to pass upward through it required a powerful pressure, and this not only produced an intense agitation among the dusty particles, 75 but lifted them away from each other and prevented the cementation which I attain.

The fineness of the particles requires that the stratum should be thin; this also acting, as above described, to relieve the mass of 80 heat before it rises to the degree where hard indurated silicates are formed. Ores of the class referred to herein include "flue dust" from iron blast furnaces and in many cases it will be found that there has passed from 90 the furnace carbon with the ore dust.

After the combustion has ceased the sintered and partly smelted porous cake or block is subjected to externally applied heat to complete the smelting operation. Considerable economy results when this final smelting operation can be carried on immediately after sintering while the cakes or blocks still retain the heat of the sintering combustion. 95 100

While I have described my invention as especially adapted for the treatment of metal bearing ores, it will be understood that it is not necessarily so limited and that it may also be used in the treatment of non-metallic 105 materials, as for instance, in the burning or roasting of cement clinkers.

What I claim is:—

1. The herein described process of treating metal oxid ores which are initially in a fine or pulverulent condition, to form uniformly porous coherent thin agglomerated or sintered masses for introduction to the blast furnace, it consisting in forming a stratum or layer of such oxids together with commingled pulverulent carbonaceous matter, said stratum being made thin to prevent the conserving of heat above a predetermined degree, igniting the carbonaceous matter at the exposed surface of the stratum, passing currents of combustion gas through the said stratum, causing the formation of carbon oxids within the mass, changing the degree of oxidation of the metal while in the presence of the carbon oxids 110 and causing the metalliferous particles to unite and cohere at the time of the oxid transformation, and at a temperature below that of the silicification of the metal. 115 120 125

2. The herein described process of form- 130

ing an agglomerated mass of metal oxide, which consists in commingling a mass of fine material carrying metal oxide and a mass of pulverized carbonaceous material, 5 forming a relatively thin layer of substantially uniform depth of this mixture, igniting the carbonaceous ingredient thereof at the top of the layer, causing the zone of ignition to propagate downward through 10 the layer by a current of air, causing reactions to take place between the carbon oxide formed by the combustion of the carbon and metallic oxide at temperatures maintained below the temperature of formation of metal 15 silicates, whereby the layer of material is transformed into cellular agglomerated masses united by the metal oxides contained, and free from metal silicates.

3. The herein described process of treating 20 pulverulent iron ores containing oxides, lower in oxygen than ferrite to form uniformly porous solid coherent cakes or blocks, it consisting in forming a relatively thin stratum of the iron oxides commingled with 25 pulverulent carbonaceous material, igniting the carbon at the exposed surface of the said stratum, passing currents of air through the said stratum from the surface of ignition, causing the combustion to pass 30 to and through the interior of the said mass, causing the iron oxides to be oxidized to an extent equivalent to that of ferrite, and while the ferrite particles are in contact, permitting them to cohere at the time of 35 action to form the agglomerated blocks or cakes as aforesaid.

4. The process of forming uniformly porous blocks or cakes from pulverulent iron oxide ore which consists in forming a 40 relatively thin stratum of the said pulverulent ore while commingled with pulverulent carbonaceous material, igniting the carbon at the exposed surfaces, passing streams of air therethrough, forming bodies 45 of carbon oxides in the mass, causing said carbon oxides to effect the deoxidizing and the oxidizing of the iron oxides and simultaneously causing the cementation of the oxides and commingled particles, substantially as described.

5. The herein described process of forming 55 an agglomerated mass of metal oxides, which consists in commingling a mass of fine material carrying metal oxide and a mass of pulverized carbonaceous material, 60 forming the resulting mixture into a relatively thin layer of substantially uniform depth, igniting the carbonaceous ingredient thereof, causing the resulting zone of 65 fusion and reaction to propagate downward through the layer by a down-draft of air, causing reactions to take place between the carbon oxides formed by the combustion of the carbon and the metallic oxides during 70 fusion at temperatures maintained below

the formation temperature of metal silicates, whereby the layer of material is transformed into cellular agglomerated masses united by the metal oxides contained, and free from metal silicates.

6. The herein described process of forming 75 an agglomerated mass of iron ferrite, which consists in commingling a mass of iron oxides and a mass of pulverized carbonaceous material, then forming the resulting mixture 80 into a relatively thin layer of uniform depth, igniting the carbonaceous ingredient at the top of the layer, causing the zone of ignition and reaction to propagate downward through the mass by a current of air, causing a partial reduction of more or less 85 of the oxides and a combining of the relatively lower with the relatively higher oxides into masses of iron ferrite, and maintaining the temperature of ignition and 90 reaction at points below the formation temperature of iron silicates, whereby the layer of material is formed into cellular agglomerated masses free from iron silicates.

7. The process of treating metal bearing 95 ore initially in a relatively fine condition and substantially free from combustible elements to prepare it for smelting, which consists in mixing with the ore a quantity of combustible substance, disposing the resulting mixture in a mass, igniting the combustible substance in the mass at one surface thereof, causing a supporter of combustion to pass from the surface of ignition to the interior and through the mass whereby combustion is made to progress into and through 100 the mass to cause sintering thereof into a cake, holding all of the particles of the mass against agitation or movement in relation to each other during combustion and sintering, and supplying to the ore before the 105 smelting action a quantity of fluxing material.

8. The herein described process of sintering 110 a mixture of fine metal-bearing material and carbonaceous matter to prepare the metal for subsequent smelting, which consists in disposing the mixture in a thin layer permeable to air, igniting the carbonaceous constituent of the mixture at a surface of 115 the mass, and causing combustion thereof to proceed entirely through the mass while the particles are held in a state of substantial quiescence among themselves, whereby there are formed uniformly cellular rigid masses 120 containing the metal.

9. The method of sintering fine ore or material, consisting in mixing such material with fine carbonaceous fuel, disposing the mixture in layer form, moving the layer 125 without substantial disturbance thereof, igniting the carbonaceous fuel of the layer, and burning out the fuel and thereby sintering the ore into a cellular structure as it is carried along.

10. The method of sintering fine ore material, consisting in mixing the same with fine carbonaceous fuel, feeding the mixture on to a bed or conveyer, and sintering the ore by complete combustion of the intermingled carbonaceous fuel as the material is carried along. 15
11. The method of sintering fine ore material, consisting in mixing it with fine carbonaceous fuel, feeding the mixture on to a moving bed or conveyer, and burning out the carbonaceous fuel under a down-draft action during travel of the mixture. 20
12. The method of sintering fine ore material, consisting in mixing it with fine carbon, feeding the mixture upon a moving conveyer, igniting the carbonaceous fuel at one point in its travel, and drawing gases down and out of the layer as the mixture is carried along beyond the ignition point.

In testimony whereof I affix my signature, in presence of two witnesses.

ARTHUR S. DWIGHT.

Witnesses:

CHARLES L. MONTAGUE,  
JOHN KNOX.

## DISCLAIMER

1,254,316.—*Arthur S. Dwight*, New York, N. Y. PROCESS OF TREATING ORES. Patent dated January 22, 1918. Disclaimer filed October 21, 1931, by the assignee, *Dwight & Lloyd Sintering Company, Inc.*

Hereby enteres this disclaimer to claims 4 and 8 of said Letters Patent, which are in the following words, to-wit:

“4. The process of forming uniformly porous blocks or cakes from pulverulent iron oxid ore which consists in forming a relatively thin stratum of the said pulverulent ore while commingled with pulverulent carbonaceous material, igniting the carbon at the exposed surfaces, passing streams of air therethrough, forming bodies of carbon oxids in the mass, causing said carbon oxids to effect the deoxidizing and the oxidizing of the iron oxids and simultaneously causing the cementation of the oxids and commingled particles, substantially as described.”

“8. The herein described process of sintering a mixture of fine metal-bearing material and carbonaceous matter to prepare the metal for subsequent smelting, which consists in disposing the mixture in a thin layer permeable to air, igniting the carbonaceous constituent of the mixture at a surface of the mass, and causing combustion thereof to proceed entirely through the mass while the particles are held in a state of substantial quiescence among themselves, whereby there are formed uniformly cellular rigid masses containing the metal.”

[*Official Gazette November 17, 1931.*]